

June 12, 1923.

1,458,222

J. F. DIETER

METHOD OF GATING CASTINGS

Filed July 18, 1921

*Fig. 1.*



*Fig. 2.*



James F. Dieter <sup>Inventor</sup>  
By his Attorneys,  
Redding & Greeley

Patented June 12, 1923.

1,458,222

# UNITED STATES PATENT OFFICE.

JAMES F. DIETER, OF HIGHLAND PARK, NEW JERSEY, ASSIGNEE TO INTERNATIONAL MOTOR COMPANY, OF NEW YORK, N. Y., A CORPORATION OF DELAWARE.

## METHOD OF GATING CASTINGS.

Application filed July 18, 1921. Serial No. 485,606.

To all whom it may concern:

Be it known that I, JAMES F. DIETER, a citizen of the United States, residing at Highland Park, in the State of New Jersey, <sup>5</sup> have invented certain new and useful Improvements in Method of Gating Castings, of which the following is a specification, reference being had to the accompanying drawing, forming a part hereof.

<sup>10</sup> This invention relates to an improved method of gating castings of metal of low specific heat and particularly aluminum, and for convenience in the specification and claim wherein reference will be made to <sup>15</sup> aluminum, it will be understood that any other metal which presents similar problems in casting is contemplated as an equivalent.

The properties of aluminum are such that <sup>20</sup> it cannot be cast readily because of the rapid rate of cooling. In different parts of such castings it has heretofore been very difficult to secure a uniform rate of cooling with the result that one part has often cooled more <sup>25</sup> readily than another and resulting stresses produce cracks or porosity. To meet this condition makeshifts have been employed in the form of chills embedded or rammed in the cores or molds and these chills have <sup>30</sup> usually been placed in the core box at points where it was desirable to accelerate the cooling to keep pace with cooling at other points. For instance, it has been the practise to place chills where the bulk of metal <sup>35</sup> is greatest. The initial expense of making these chills, the labor of installing them and the cost of replacement has made their use very undesirable and it is believed that unfavorable conditions in the casting itself are <sup>40</sup> apt to be created by the presence of chills.

In the usual method of gating, risers are placed near the heaviest metal parts and communicate with the mold. These risers serve the purpose of supplying a head or <sup>45</sup> pressure to the metal in the mold and also a reserve to fill up the space left by contraction in cooling. Since the metal entering the risers flows from the mold and is the first metal poured, relatively speaking, it <sup>50</sup> is natural that it should become somewhat chilled before reaching the risers and have a tendency to freeze therein. This condition, particularly in the casting of aluminum, defeats one of the principal purposes of the

metal in the risers since it does not constitute a hot and effective reserve. <sup>55</sup>

In accordance with the improved method chills are eliminated and yet such conditions are set up as will insure a uniform cooling throughout the mold, all parts of the <sup>60</sup> casting being maintained at a sufficient high temperature, during the cooling, by the hot metal within the risers. To accomplish this the risers are gated in the runners. The metal is fed in uniformly through the pouring basin and passes through the runners to the mold. The risers are gated in the runners so that the metal ultimately held in reserve therein is the last metal poured and hence the hottest. This hot metal effectively <sup>65</sup> in maintaining the temperature throughout the casting so that it will be caused to cool uniformly. There is illustrated in the accompanying drawing in somewhat diagrammatic form a gate embodying the invention. <sup>70</sup>

In the drawing—

Figure 1 is a view in plan of a flask showing the risers into the runners.

Figure 2 is a view in vertical section through the flask shown in Figure 1 and taken along the planes indicated by the broken lines 2—2 of Figure 1 and looking in the direction of the arrows. <sup>80</sup>

As the description proceeds it will be evident that not only is the invention not limited to the character of the metal employed in casting but, further, is not limited to the type of casting or flask. Variations in the form and disposition of the pouring basins, runners and risers will suggest themselves to one skilled in the foundry art and be adapted to prevailing conditions. <sup>85</sup>

The flask *a* is shown as including a mold for any suitable casting. The pouring basins *b*, two in number, have communicating therewith the runners *c* through which the metal flows to the mold and in these runners are gated risers *d* in such number and position as will be most effective for their intended purpose. <sup>95</sup>

Heretofore the risers have not been gated into the runners so that the metal reaching them has necessarily traversed the mold. The tortuous paths taken have tended to chill the metal and since this metal has been the first poured, it has not been hot, relatively speaking, when finally within the risers. Such condition has defeated, to a <sup>100</sup> <sup>105</sup>

large extent, the very purpose of the risers since the metal therein has not been in a condition to supply a head or pressure and fill up the space left by contraction in cooling. Of course with metals, like aluminum, of low specific heat the effect has been accentuated to a point where freezing has occurred.

In accordance with the present invention 10 the method of gating is such that contrary conditions are realized. The metal flows freely along the runners into the mold and the last poured metal enters the risers. This 15 metal is therefore the hottest and serves to maintain within the body of the casting a uniform temperature during cooling and insure uniform contraction while continuously

filling up the spaces left by such contraction. No chills are necessary and yet, in practise, better castings have been secured than before. 20

I claim as my invention:

The herein described method of casting comprising forming a riser in communication with the runner, and between the pouring basin and the mould proper, whereby the riser fills with the last poured metal, which metal feeds into, and exerts pressure on, the metal in the mould during the cooling thereof. 25 30

This specification signed this ninth day of July, A. D. 1921.

JAMES T. DIETER.